

## UNITED STATES PATENT OFFICE

2,111,769

## LUBRICATING COMPOSITIONS

George De Witt Graves, Wilmington, Del., assignor to E. I. du Pont de Nemours & Company, Wilmington, Del., a corporation of Delaware

No Drawing. Application June 15, 1934,  
Serial No. 730,783

20 Claims.

(Cl. 87—9)

This invention relates to the preparation of improved lubricating oils, and particularly to the preparation of new compositions of matter which effect improvements in certain qualities of lubricating oils when added thereto.

Most of the lubricating oils used in the United States contain saturated paraffin hydrocarbon waxes as naturally occurring components. The presence of these paraffins in limited quantities imparts desirable qualities to the lubricating oils. However, the waxy hydrocarbon materials raise the pour-point of the oils to values that make them unsatisfactory for use at lower winter temperatures. There are methods used at the present time for reducing the pour-point of lubricating oils which ordinarily consist of freezing the oil and separating the solidified paraffin or other waxy material by filtration or by centrifugal action. These methods are costly and may adversely affect other desirable qualities of the oil such as its viscosity-temperature characteristics.

Other more satisfactory methods of reducing the pour-point of lubricating oils have been developed. In general, they involve the addition of certain compounds to the oils which permit the retention of the desirable paraffinic material but give the oils a low pour-point and exert a favorable influence on the viscosity-temperature characteristics. U. S. Patent No. 1,815,022 is typical of several patents relating to these pour-point depressants.

This invention has as an object the production of high-grade lubricating oils having the desirable property of low pour-point. A further object of the invention is the production of new compositions of matter which, in addition to oils suitable only for summer use, will transform them to products suitable also for winter use. Other objects will appear hereinafter.

These objects are accomplished by the following invention wherein a lubricating oil containing a solid waxy constituent in proportion sufficient to give a relatively high pour-point, is blended with a high molecular weight ether containing material such as a dehydration condensation polymer of octadecanediol, or a condensation product of a chlorinated paraffin with an ether of a polycyclic phenol.

The process of the present invention is illustrated in the examples given below which are not to be regarded as limitative. The "standard oil" referred to in the examples was a commercial heavy duty engine oil, representative of a summer grade oil, and contained both paraffin wax

and petroleum wax. Its pour-point was 25° F. The pour-points outlined in this specification were determined according to the procedure outlined in Technical Paper 323-A of the Bureau of Mines, p. 36 of the 1924 edition.

5

## Example 1

To a solution of 13.5 g. of the ethyl ether of betanaphthol in 19 g. of cyclohexane was added 10 g. of anhydrous aluminum chloride. Considerable heat was developed, and the aluminum chloride turned black. The temperature was lowered to 35° C., and 90 g. of chlorinated paraffin wax (12% chlorine) was stirred in. Stirring was continued for about 23 hours, after which 15 the temperature was raised to 80°—85° C., and held for one-half hour. There was considerable semi-solid material present, so 200 g. more of cyclohexane was added to promote filtration. The solution was in part decanted and in part 20 filtered from the sludge. After a vacuum distillation to remove the solvent, there was obtained 44 g. of a waxy, heavy oil. Small quantities of the product were added to the "standard oil" mentioned above to test its properties as a pour-point depressant.

10

15

20

25

30

35

| Percent by weight added | Pour-point of "standard oil"—degrees F. |
|-------------------------|-----------------------------------------|
| 0.0                     | +25                                     |
| 0.25                    | +20                                     |
| 0.50                    | +5, +15, +15                            |
| 1.0                     | 0, -5                                   |
| 2.0                     | -5, -5                                  |

It will be apparent from the table that the condensation product is most efficient when added to the extent of 1%. Further additions continue to lower the pour-point, but only to a relatively small degree.

## Example 2

A high melting paraffin or petroleum type wax averaging 40 carbon atoms per molecule was chlorinated to the mono-halide stage (7% chlorine) on a steam bath. Condensation of the chlorinated wax with alpha-naphthol methyl ether in cyclohexane, as described in Example 1, yielded a product quite solid at room temperature. One per cent of the material lowered the pour-point of the "standard oil" to +5° F.

45

50

## Example 3

Ten grams of diphenylene oxide dissolved in 55

cyclohexane was condensed with 90 g. of the chloroparaffin above described, using aluminum chloride as the condensing agent. The product was a soft wax at room temperature. It was 5 tested as a pour-point depressant without distilling off any residual chloroparaffin. Two per cent of the crude material lowered the pour-point of the "standard oil" to 0° F.

10 *Example 4*

10 Forty-four grams of pure octadecanediol and 0.3 g. of sodium hydroxide were heated at 235°-240° C. at 20 mm. pressure for 88 hours. The temperature was then raised to 260°-275° C. and 15 the heating continued under 15 mm. pressure for 76 hours. During the latter heating period samples were removed from time to time, and their pour-point depressant qualities tested. The following table shows the effects of adding 1% of 20 the octadecanediol condensation product to the "standard oil".

|    | Hours at<br>260°-275° C. | Pour-point<br>degrees F. |
|----|--------------------------|--------------------------|
| 25 | 21                       | +20                      |
|    | 45                       | +10                      |
|    | 53                       | +15                      |
|    | 69                       | 0                        |
| 30 | 76                       | -5                       |

Example 5

35 Fifty grams of the crude products obtained by the hydrogenation of castor oil, and containing a substantial quantity of octadecanediol, was heated with 1.25 g. of sodium hydroxide for 63.5 hours at 260°-275° C. and 13 mm. pressure. The condensation product when cool was a jelly-like, colorless solid. The following table indicates the effects 40 upon the pour-point of the "standard oil" obtained by the addition of various quantities of the condensation product.

|    | Percent of<br>product<br>added | Pour-point of<br>"standard oil"—<br>degrees F. |
|----|--------------------------------|------------------------------------------------|
| 45 | 0.0                            | +25                                            |
|    | 0.25                           | +15                                            |
|    | 0.50                           | +5, 0                                          |
| 50 | 1.0                            | 0, -5                                          |

In preparing the wax for the condensation, any paraffin or petrolatum type wax, either pure or in the mixed state, may be chlorinated. The chlorination may be effected by well-known methods, preferably to the mono-halide stage, although it may be carried further, if desired. Although condensation products of only three specific polycyclic phenol ethers have been described in the examples, other polycyclic ethers may be used such as mixed cyclic ethers of the class comprising naphthyl ethers of monohydric alcohols and phenois such as propyl, butyl, amyl, dodecyl and phenyl; aliphatic or aromatic ethers of polycyclic hydroxy naphthalenes, di-naphthol, of hydroxy anthracenes, and of mono or polyhydroxy diphenyls. In effecting the condensation reaction, the ratio by weight of the chlorinated product to the ether may be varied considerably. During the reaction, constant agitation is desirable, and an inert solvent such as cyclohexane should be used. To facilitate the condensation, a temperature of 30°-40° C. is desirable, although room temperature may be employed with a correspondingly longer time. It is desirable to raise the

temperature slowly to 80°-100° C., after the reaction subsides, not only to insure completion of the reaction, but to drive out hydrochloric acid vapors from the mixture.

The condensation products prepared as described in the examples may, in some instances, contain unreacted chloro-paraffin and various by-products which are not active as pour-point depressants. The crude products may be used directly or the active material may be extracted 10 with solvents such as ethylene dichloride, ethyl methyl ketone, acetone, etc. to obtain a more active product. It is to be noted that the pour-point depressants of the present invention are high molecular weight ethers containing a plurality of aromatic nuclei and/or ether groups. 15

The pour-point depressants of the present invention may be added to lubricating oils in any desirable proportion. Generally the preferred quantity for pour-point depression will be 0.25- 20 2.0%. Larger quantities may be used but are not in general economical.

The pour-point depressants of the present invention are valuable additions to the group of known pour-point depressants. The preparation 25 of these depressants is, in general, practical and economical, and the process is of considerable technical and economic importance in view of the fact that by the use of such depressants lubricating oils may be made of utility within a wider 30 range of temperature.

The above description and examples are intended to be illustrative only. Any modification of or variation therefrom which conforms to the spirit of the invention is intended to be included 35 within the scope of the claims.

I claim:

1. An improved lubricating oil comprising a viscous petroleum hydrocarbon fraction containing a solid waxy constituent in proportion sufficient to give a relatively high pour-point blended with 0.25 to 2.0% of a high molecular weight ether condensation product containing a long aliphatic hydrocarbon chain. 40

2. An improved lubricating oil comprising a viscous petroleum hydrocarbon fraction containing a solid waxy constituent in proportion sufficient to give a relatively high pour-point blended with 0.25 to 2.0% of a high molecular weight ether containing material of the class consisting of octadecanediol condensation polymers and condensation products of halogenated high molecular weight paraffins with a polycyclic aryl ether of the class consisting of alkyl and aryl naphthyl ethers, ethers of polyhydroxy naphthalenes, ethers of dinaphthol, ethers of hydroxy anthracenes, and ethers of mono and polyhydroxy diphenyls. 55

3. An improved lubricating oil comprising a viscous petroleum hydrocarbon fraction containing a solid waxy constituent in proportion sufficient to give a relatively high pour-point blended with 0.25 to 2.0% of a high molecular weight ether containing material obtained by the dehydration condensation of octadecanediol. 60

4. An improved lubricating oil comprising a viscous petroleum hydrocarbon fraction containing a solid waxy constituent in proportion sufficient to give a relatively high pour-point blended with 0.25 to 2.0% of octadecanediol condensation 70 polymer.

5. An improved lubricating oil comprising a viscous petroleum hydrocarbon fraction containing a solid waxy constituent in amount sufficient to give a relatively high pour-point, blended with 75





## DISCLAIMER

2,111,769.—*George De Witt Graves, Wilmington, Del.* LUBRICATING COMPOSITIONS.  
Patent dated March 22, 1938. Disclaimer filed June 14, 1939, by the  
assignee, *E. I. du Pont de Nemours and Company*.

Hereby enters this disclaimer as to claim 1 of said patent.  
[*Official Gazette July 4, 1939.*]